

Dec. 20, 1932.

P. C. KEITH, JR.

1,891,890

METHOD OF MAKING ASPHALT

Filed July 10, 1928



Patented Dec. 20, 1932

1,891,890

# UNITED STATES PATENT OFFICE

PERCY C. KEITH, JR., OF BERNARDSVILLE, NEW JERSEY, ASSIGNOR, BY MESNE ASSIGNMENTS, TO GASOLINE PRODUCTS COMPANY, INC., OF NEWARK, NEW JERSEY, A CORPORATION OF DELAWARE

## METHOD OF MAKING ASPHALT

Application filed July 10, 1928. Serial No. 291,601.

This invention relates to the production of commercial asphalt from cracking-coil tar and will be understood from the following description read in conjunction with the drawing 5 which is an elevation principally in section of apparatus in which my method may be carried into effect.

Petroleum oil to be cracked is introduced through the pipe 1 controlled by valve 2 to 10 the tubular heater 3. The tubular heater consists of a number of sections of tubing joined end to end by cross-over connections to form a continuous circuit. It is surrounded by the refractory setting 4 and may be 15 heated through port 5 by means of the burner 6. The heating is so conducted that the material is heated to a relatively high temperature, usually above 800° F., and is then discharged through pipe 7 into the digestion 20 chamber 8. This consists of a drum, preferably surrounded by insulating material 9, in which the cracked petroleum oil is retained for a further period during which cracking reactions proceed, principally as a 25 result of the contained heat. The precise form of tubular heater and digestion drum are unimportant; any alternative type may be employed in place of those specifically illustrated. The tubular heater is known in 30 the trade as a cracking coil and will be herein-after referred to as such. Ordinarily the coil and drum operate under pressure considerably in excess of atmospheric, frequently as high as several hundred pounds gauge, which 35 may be reduced at the outlet 10 by a reduction valve such as 11. The cracked material which is continuously abstracted from the digestion drum is introduced at reduced pressure, say 15 pounds gauge or less, into the low 40 pressure drum 12 through the pipe 11a. The cracked material is preferably discharged into this drum through a perforated pipe such as 13. Separation takes place in the drum 12, tarry material collecting in the lower part 45 thereof while vapors which are substantially tar free pass off overhead through the pipe 14. When operating under extremely high pressures in the coil and drum, or during vapor phase operation, it is frequently advisable to 50 introduce petroleum oil with the cracked

material, which may be done by means of the oil inlet pipe 15 controlled by valve 16 and discharging into pipe 11a. While any oil introduced in this manner will absorb the super-heat of the cracked material and control the consistency of the tar produced, it is desirable to introduce through the pipe 15 an oil containing tar-forming constituents which will add to the tar produced by cracking and the additional benefit will be simultaneously derived in separating the tar-forming constituents from the oil so introduced. The vapor passing off through 14 enters the rectifying column 17. This consists of any suitable type of rectifying equipment; that shown is provided with the conventional partitions which carry over-flow pipes and vapor distributors of any suitable character, not shown. Condensation is produced by cooling coils in the upper part of the tower, such as 18 and 19. The coil 19 may conveniently be supplied with oil for the cracking coil which is thereby pre-heated prior to cracking. The total amount of cooling obtained by the use of coils 18 and 19 is preferably so controlled that the final vapor passing off through the pipe 20 consists essentially of gasoline which may then be condensed and worked up for the market in any approved manner. A liquid bottoms collects in the 70 base of the tower 17 and is preferably withdrawn continuously through the pipe 21 and pumped by means of the pump 22 through the pipe 23 controlled by valve 24 back into the cracking coil, thereby recirculating the 75 said bottoms and adding to the total quantity of gasoline produced. The drum 12 is preferably surrounded by insulation 12a and the tar collecting in this drum is withdrawn continuously or periodically by means of the pipe 25 controlled by valve 26 and thereby discharged into the intermediate portion of the stripping drum 27. The pipe 25 is preferably surrounded by insulation 26a so that the tar may be introduced substantially without loss of heat into the intermediate portion of the drum 27. This drum carries horizontal partitions 28 equipped with the customary vapor distributors and over-flow pipes, not shown, below the point of introduc- 80 85 90 95 100

tion of the said tar. A coil 30 is provided in the base of the drum 27 to supply additional heat if necessary and steam may be introduced by means of the pipe 31 controlled by 5 the valve 32 and terminating in the distributor 33. The drum 27 preferably carries foraminous plates 34 above the point of introduction of the tar, which may in turn carry tile or other baffling means, not shown, to 10 knock down entrainment from the ascending vapor. Vapors may be conducted from the drum 27 through the vapor pipe 36 which discharges into the condenser 37. This condenser consists of an elongated drum provided 15 with water inlet 38 at the lower end and water outlet 39 at the upper end. A number of tubes 42 are arranged within the drum between the two header plates 40 and 41 so that the water circulates within the tubes 42. 20 Any oil vapor discharged by the pipe 36 circulates in the space external to the tubes and is thereby condensed. The condensate is continuously withdrawn through the pipe 44 discharging into the accumulator 45 from 25 which it may be continuously or periodically withdrawn by means of the pipe 46 connected to the pump 47 and thereby diverted through the pipe 48 to any suitable accumulator. By means of the pipe 49 connected to the accumulator 45 and the vacuum pump 50 the condenser 37 and drum 27 are maintained under 30 vacuum. The vacuum pump 50 may be of any suitable type although that illustrated diagrammatically is barometric. The operation 35 of the cracking coil will be obvious to those familiar with the art. In operating the equipment for the reduction of the tar produced by the cracking equipment a vacuum is applied through the condenser 37 to the 40 tar discharged into the drum 27. I preferably employ a vacuum corresponding to an absolute pressure of less than 100 mm. of mercury. This automatically results in a considerable reduction of the tar delivered 45 by the pipe 25. In consequence of the retained heat of the tar this is distinctly assisted by the fact that the tar when brought from the cracking system may be at a temperature of 700° or 800° F. The reducing effect of 50 the vacuum applied to the heated tar is further augmented by the stripping effect of the steam introduced through the distributor 33 and the additional heat applied by means of the coil 30. The coil 30 is preferably supplied 55 with super-heated steam for this purpose. The effect of these agencies is so controlled as to produce a liquid residuum in the bottom of the drum 27 corresponding to a commercial asphalt. By means of the overflow 60 pipe 51 the level of this material in the bottom of the drum 27 is maintained above the coil 30, any excess being continuously diverted through the overflow pipe 51 controlled by valve 52 and transferred by means of the 65 pump 53 to any suitable accumulator. The

grade of material produced may conveniently include all of those products which are generically covered by the term asphalt and which range from the liquid or semi-liquid products known as binders down to the products which are solid at normal temperatures and which constitute asphalts of relatively high melting point and low penetration. 70

The foregoing specific illustration of my method is by way of illustration and not of limitation. It is my intention that the invention be limited only by the appended claims, or their equivalents, in which I have endeavored to cover broadly all inherent 75 novelty. 80

I claim:

1. The method of reducing tar residuum produced by heating petroleum oil, under pressure, in a confined stream to a cracking temperature, retaining the cracked material, under pressure, in a digestion zone, continuously withdrawing cracked material from the digestion zone and discharging it into a zone maintained under reduced pressure to produce a first vapor and a tar residuum, which comprises continuously discharging the tar residuum without substantial loss of heat into a zone maintained under vacuum, stripping the material in said zone maintained under vacuum to the extent necessary 90 to produce a residuum of commercial asphalt. 95

2. The method of reducing tar residuum produced by heating petroleum oil, under pressure, in a confined stream to a cracking temperature retaining the cracked material, under pressure, in a digestion zone, continuously withdrawing cracked material from the digestion zone and discharging it into a zone maintained under reduced pressure to produce a first vapor and a tar residuum which comprises continuously discharging the tar residuum without substantial loss of heat into a zone maintained under vacuum to produce a second vapor and a liquid residuum, contacting the liquid residuum counter-currently with steam to the extent necessary to produce a residuum of commercial asphalt. 105 110

3. The method of reducing tar residuum produced by heating petroleum oil, under pressure, in a confined stream to a cracking temperature, retaining the cracked material, under pressure, in a digestion zone, continuously withdrawing cracked material from the digestion zone and discharging it into a zone maintained under reduced pressure to produce a first vapor and a tar residuum which comprises continuously discharging the tar residuum without substantial loss of heat into a zone maintained under vacuum to produce a second vapor and a liquid residuum, heating the liquid residuum in said zone maintained under vacuum and counter-currently contacting steam therewith to the extent necessary to produce a residuum of commercial asphalt. 115 120 125 130

4. The method of making asphalt which comprises heating petroleum oil under pressure in a confined stream to a cracking temperature, retaining the cracked material under pressure in a digestion zone, continuously withdrawing cracked material from the digesting zone, combining therewith petroleum oil containing tar-forming constituents, discharging the combined materials into a zone maintained under reduced pressure to produce a first vapor and a tar residuum and continuously withdrawing the tar residuum without substantial loss of heat to strip the same to produce a residuum of commercial asphalt.
5. The method of making asphalt which comprises heating petroleum oil under pressure in a confined stream to a cracking temperature, retaining the cracked material under pressure in a digestion zone, continuously withdrawing cracked material from the digesting zone, combining therewith petroleum oil containing tar-forming constituents, discharging the combined materials into a zone maintained under reduced pressure to produce a first vapor and a tar residuum, continuously withdrawing the tar residuum and discharging the same without substantial loss of heat into a zone maintained under vacuum, stripping the tar residuum in said zone maintained under vacuum to the extent necessary to produce a residuum of commercial asphalt.

In testimony whereof, I have signed my name to this specification this 5th day of July, 1928.

PERCY C. KEITH, JR.

40

45

50

55

60

65